

# UNITED STATES PATENT OFFICE.

BENJAMIN DAWSON PORRITT, OF EDINBURGH, SCOTLAND, ASSIGNOR TO THE NORTH  
BRITISH RUBBER COMPANY LIMITED, OF EDINBURGH, SCOTLAND.

## BALLOON FABRIC AND THE LIKE.

1,118,149.

Specification of Letters Patent. Patented Nov. 24, 1914.

No Drawing.

Application filed February 11, 1913. Serial No. 747,777.

To all whom it may concern:

Be it known that I, BENJAMIN DAWSON PORRITT, a subject of the King of the United Kingdom of Great Britain and Ireland, and 5 resident of Edinburgh, Scotland, have invented certain new and useful Improvements in Balloon Fabrics and the like, of which the following is a specification.

Balloon fabrics constructed with a layer 10 of rubber to insure gas holding qualities have been known for a considerable time and have been extensively used. It is well known that two points require special attention to secure a satisfactory result and 15 durability. The rubber used for the impermeable layer must be of the highest quality, and it must be protected, by some covering, from the actinic rays which are very intense in the higher regions of the atmosphere 20 and cause rapid deterioration and oxidation of the proofing. It is a known fact that metals of high atomic weight such as lead possess the power of stopping radiations of short wave length, and this property is 25 made use of in X-ray work and with mercury vapor lamps.

The present invention consists in the application of this principle to balloon fabrics and the like combined with the other methods of protection which have already been 30 used for the purpose.

The proofing which we use is one composed of litharge, bismuth oxid or other heavy metallic oxid, sulfur necessary for 35 vulcanization and rubber, and a thin layer of this is applied as a coating to the outside of the fabric.

The following example illustrates my invention:

40 *Fabric.*—Two plies preferably of Sea Island cotton are used, the outer ply being dyed yellow with lead chromate or a yellow die fast to light, and if considered necessary, biased to obviate tearing of the fabric.

45 *Proofing.*—Between these two plies of fabric is placed the layer most important for securing gas tightness—such layer consisting of a mixing suitable for the purpose. On the back of the two ply fabric a light 50 layer of a similar proofing is spread to protect the inner fabric from the action of moisture deposited by the gas on passing from warmer to colder regions. Between

the two plies and next the outer or yellow fabric a thin layer of proofing containing yellow pigment is placed, thus serving to further cut off light from the blue region of the spectrum. For this purpose inorganic coloring matters are most suitable. On the outside of the fabric the important 55 protecting layers are placed. Next the yellow cloth is a thin layer of proofing containing litharge or other heavy oxid of a percentage composition most suitable for the purpose. On the surface of this proofing 60 fine aluminum powder is dusted. This serves to reflect a large proportion of the light and heat waves and thereby serves the double purpose of minimizing the risk of perishing due to actinic action and also 65 preventing the sudden expansion of the gas in the envelop, which expansion might otherwise occur on emerging from a cloud into sunshine. The whole is firmly united 70 together and vulcanized in any known manner, either by heat or chlorid of sulfur in 75 the cold.

The fabric consists, therefore, of the following 7 layers:—(1) Aluminium dust to reflect light and heat waves. (2) Heavy 80 metallic oxid proofing to absorb actinic light. (3) Dyed fabric—biased if necessary—further reducing actinic action. (4) Layer of yellow proofing. (5) Impermeable layer of proofing. (6) Layer of undyed fabric. 85 (7) Layer of proofing to protect this from the injurious effects of moisture.

### Claims:

1. An improved balloon fabric or the like having, applied thereto, a light ray proofing 90 composed of a heavy metallic oxid and rubber.

2. An improved balloon fabric, or the like having, applied thereto, a light ray proofing composed of a heavy metallic oxid, sulfur 95 and rubber.

3. An improved balloon fabric, or the like, consisting of an outer ply dyed yellow, an inner ply, a gas-tight layer between the plies and a light ray proofing, on the outside of 100 these plies containing a heavy metallic oxid.

4. An improved balloon fabric, or the like, consisting of an outer ply, an inner ply, a gas-tight layer between the plies, a gas-tight layer on the inner surface of the inner ply, 105 a proofing containing a heavy metallic oxid

on the outside of the outer ply and an aluminium powder dusting on the said proofing.

5. An improved balloon fabric or the like consisting of a dyed fabric, a heavy metallic oxid proofing on the dyed fabric, aluminium dust on the proofing, a layer of yellow proofing on the opposite side of the dyed fabric,

a layer of air-tight proofing on the yellow proofing, a layer of undyed fabric next the 10 air-tight proofing, and a layer of proofing on the undyed fabric.

BENJAMIN DAWSON PORRITT.

Signed in presence of—

THOMAS HERBERT PORRITT,

JAMES WHITELAW.